



US011560614B2

(12) **United States Patent**  
**Yoshitomi et al.**

(10) **Patent No.:** **US 11,560,614 B2**  
(45) **Date of Patent:** **\*Jan. 24, 2023**

(54) **HIGH-STRENGTH GALVANIZED STEEL SHEET, HIGH STRENGTH MEMBER, AND METHOD FOR MANUFACTURING THE SAME**

(71) Applicant: **JFE Steel Corporation**, Tokyo (JP)

(72) Inventors: **Hiromi Yoshitomi**, Tokyo (JP); **Masaki Koba**, Tokyo (JP); **Tatsuya Nakagaito**, Tokyo (JP); **Yoshitsugu Suzuki**, Tokyo (JP)

(73) Assignee: **JFE Steel Corporation**, Tokyo (JP)

(\*) Notice: Subject to any disclaimer, the term of this patent is extended or adjusted under 35 U.S.C. 154(b) by 143 days.

This patent is subject to a terminal disclaimer.

(21) Appl. No.: **17/041,830**

(22) PCT Filed: **Mar. 29, 2019**

(86) PCT No.: **PCT/JP2019/014234**

§ 371 (c)(1),

(2) Date: **Sep. 25, 2020**

(87) PCT Pub. No.: **WO2019/189848**

PCT Pub. Date: **Oct. 3, 2019**

(65) **Prior Publication Data**

US 2021/0025045 A1 Jan. 28, 2021

(30) **Foreign Application Priority Data**

Mar. 30, 2018 (JP) ..... JP2018-068995  
Mar. 1, 2019 (JP) ..... JP2019-037384

(51) **Int. Cl.**

**C22C 38/54** (2006.01)

**C21D 9/46** (2006.01)

(Continued)

(52) **U.S. Cl.**  
CPC ..... **C22C 38/54** (2013.01); **C21D 8/0205** (2013.01); **C21D 8/0226** (2013.01);  
(Continued)

(58) **Field of Classification Search**

None  
See application file for complete search history.

(56) **References Cited**

U.S. PATENT DOCUMENTS

2016/0214351 A1 7/2016 Harako et al.

2017/0044640 A1 2/2017 Kimura et al.

(Continued)

FOREIGN PATENT DOCUMENTS

EP 2716773 A1 4/2014

EP 3173494 A1 5/2017

(Continued)

OTHER PUBLICATIONS

Chinese Office Action with Search Report for Chinese Application No. 201980023156.2, dated Sep. 16, 2021, 10 pages.

(Continued)

*Primary Examiner* — Anthony M Liang

(74) *Attorney, Agent, or Firm* — RatnerPrestia

(57) **ABSTRACT**

A high-strength galvanized steel sheet includes a steel sheet having a chemical composition containing a predetermined component element, a mass ratio of a content of Si to a content of Mn in the steel (Si/Mn) being 0.1 or more and less than 0.2, and the balance: Fe and incidental impurities, and a steel structure in which an average grain size of inclusions containing at least one of Al, Si, Mg, and Ca and existing in an area extending from a surface to a position of  $\frac{1}{3}$  of a sheet thickness is 50  $\mu\text{m}$  or less, and an average nearest distance between ones of the inclusions is 20  $\mu\text{m}$  or more; and a galvanized layer provided on a surface of the steel sheet, in which an amount of diffusible hydrogen contained in the

(Continued)



steel is less than 0.25 mass ppm, and a tensile strength is 1100 MPa or more.

**13 Claims, 1 Drawing Sheet**

**(51) Int. Cl.**

**C21D 8/02** (2006.01)  
**C23C 2/06** (2006.01)  
**C23C 2/26** (2006.01)  
**C22C 38/50** (2006.01)  
**C22C 38/44** (2006.01)  
**C22C 38/46** (2006.01)  
**C22C 38/42** (2006.01)  
**C22C 38/00** (2006.01)

**(52) U.S. Cl.**

CPC ..... **C21D 8/0236** (2013.01); **C21D 9/46** (2013.01); **C22C 38/002** (2013.01); **C22C 38/42** (2013.01); **C22C 38/44** (2013.01); **C22C 38/46** (2013.01); **C22C 38/50** (2013.01); **C23C 2/06** (2013.01); **C23C 2/26** (2013.01); **C21D 2211/001** (2013.01); **C21D 2211/002** (2013.01); **C21D 2211/005** (2013.01); **C21D 2211/008** (2013.01)

**(56)**

**References Cited**

U.S. PATENT DOCUMENTS

2017/0218475 A1 8/2017 Kawasaki et al.  
 2020/0032364 A1 1/2020 Hirashima et al.  
 2020/0190617 A1 6/2020 Hasegawa et al.

FOREIGN PATENT DOCUMENTS

JP 2002235160 A 8/2002  
 JP 2006037130 A 2/2006  
 JP 2011111670 A \* 6/2011  
 JP 2011111670 A 6/2011

|    |               |        |
|----|---------------|--------|
| JP | 2013163827 A  | 8/2013 |
| JP | 2017048412 A  | 3/2017 |
| JP | 6525114 B1    | 6/2019 |
| KR | 20160072898 A | 6/2016 |
| WO | 2004063410 A1 | 7/2004 |
| WO | 2015029404 A1 | 3/2015 |
| WO | 2016103535 A1 | 6/2016 |
| WO | 2018124157 A1 | 7/2018 |
| WO | 2018146828 A1 | 8/2018 |

**OTHER PUBLICATIONS**

Hasegawa et al., "Influence of Metal Structure on the Bending Formability of an Ultrahigh-strength Steel Sheet of the 980-MPa Class", CAMP-ISIJ, vol. 20 (2007), 3 pages, published by the Iron and Steel Institute of Japan.

Nakamura et al., "Influence of Structure on the Stretch Flange Moldability of an Ultrahigh-strength Cold Rolled Steel Sheet", CAMP-ISIJ, vol. 13 (2000), 11 pages, published by the Iron and Steel Institute of Japan.

Non Final Office Action for U.S. Appl. No. 17/041,680, dated May 6, 2022, 13 pages.

Non Final Office Action for U.S. Appl. No. 16/960,733, dated May 23, 2022, 27 pages.

International Search Report and Written Opinion for International Application No. PCT/JP2019/014234, dated Jun. 25, 2019, 6 pages. Kromhout, J.A. et al., "Understanding Mould Powders for High-Speed Casting", Nov. 29, 2016, vol. 45(3), 9 pages, Ironmaking & Steelmaking: Processes, Products and Applications.

Extended European Search Report for European Application No. 19 777 299.9, dated Oct. 26, 2020, 11 pages.

Korean Office Action for Korean Application No. 10-2020-7028049, dated Feb. 8, 2022, with Concise Statement of Relevance of Office Action, 8 pages.

European Communication Pursuant to Article 94(3) for European Application No. 19777299.9, dated Jun. 4, 2021, 4 pages.

Chinese Office Action for Chinese Application No. 201980023156.2, dated May 11, 2021 with Concise Statement of Relevance of Office Action, 10 pages.

Non Final Office Action for U.S. Appl. No. 17/041,743, dated Jul. 19, 2022, 8 pages.

\* cited by examiner



**HIGH-STRENGTH GALVANIZED STEEL SHEET, HIGH STRENGTH MEMBER, AND METHOD FOR MANUFACTURING THE SAME**

**CROSS REFERENCE TO RELATED APPLICATIONS**

This is the U.S. National Phase application of PCT/JP2019/014234, filed Mar. 29, 2019, which claims priority to Japanese Patent Application No. 2018-068995, filed Mar. 30, 2018 and Japanese Patent Application No. 2019-037384, filed Mar. 1, 2019, the disclosures of these applications being incorporated herein by reference in their entireties for all purposes.

**FIELD OF THE INVENTION**

The present invention relates to a high-strength galvanized steel sheet, a high strength member, and a method for manufacturing the same that are excellent in plating ability and bendability, and that is suitable for building materials and automotive collision-resistant parts, and a method for manufacturing the same.

In these days when crash safety and fuel efficiency improvement of automobiles are strongly required, the strength increase of steel sheets that are materials of parts is being advanced. Further, in view of the fact that automobiles are being widely spread on a global scale and automobiles are used for various uses in diverse areas and climates, steel sheets that are materials of parts are required to have high antirust properties.

In general, when the strength of a steel sheet is enhanced, the formability of the steel sheet is reduced. In particular, a steel sheet provided with plating tends to have poorer formability than a steel sheet not provided with plating.

If a large amount of an alloying element is incorporated in order to increase strength, it is difficult for a good quality plating film to be formed on the steel sheet. Further, it is known that, if plating of Zn, Ni, or the like is provided, hydrogen that enters during the manufacturing process is less likely to be released from the interior of the steel.

Steel sheets having excellent bendability have thus far been developed. Based on the features of the method for forming such a steel sheet, how to design a location that is exposed to most severe forming conditions at the time of bending, that is, a location where stress is concentrated is presented as a solution to an issue. In particular, in the case of a steel sheet containing two or more kinds of steel structures with different hardnesses, it is likely that deformation will concentrate and defects of microvoids will occur at the interface between steel structures, and consequently bendability is degraded.

Also the control of an atmosphere in the furnace of an annealing-plating step is attempted in order to deposit good quality plating.

In Non-Patent Literatures 1 and 2, while the steel structure of a steel sheet contains ferrite and martensite, a steel structure of ferrite and martensite is temporarily produced and then tempering is performed to soften the martensite, and bendability is improved.

Patent Literature 1 discloses a high-strength steel sheet in which a structure homogeneity index given by a standard deviation of Rockwell hardness of a surface of a steel sheet and serving as an index indicating the homogeneity of the steel sheet is 0.4 or less and that is good in ductility and bendability and has a maximum tensile stress of 900 MPa or

more, and a method for manufacturing the same. This literature provides a technique obtained as a result of improving, as a factor influencing bendability, the heterogeneity of a solidified structure at the time of casting, and presents, by this method, a steel sheet that has a maximum tensile stress of 900 MPa or more and is excellent in bendability.

In Patent Literature 1, at this time, the interior of an annealing furnace of a continuous galvanizing line is set to an atmosphere having a hydrogen concentration of 1 to 60 vol % and containing N<sub>2</sub>, H<sub>2</sub>O, O<sub>2</sub>, and incidental impurities as the balance, and the logarithm of the partial pressure of water and the partial pressure of hydrogen in the atmosphere, log (P<sub>H2O</sub>/P<sub>H2</sub>), is prescribed to  $-3 \leq \log (P_{H2O}/P_{H2}) \leq -0.5$  in order to ensure good quality plating ability.

Patent Literature 2 provides a dual-phase steel sheet that contains 50% or more of bainite and 3 to 30% of retained austenite and in which the ratio between the hardness Hvs of an outer layer of the steel sheet and the hardness Hvb of a portion of  $\frac{1}{4}$  of the thickness of the steel sheet is prescribed to 0.35 to 0.90. Further, annealing is performed in an atmosphere in which log(partial pressure of water/partial pressure of hydrogen) is -3.0 to 0.0, and thereby plating ability is ensured in a high alloy system.

Patent Literature 3 ensures bendability by prescribing a decarburized ferrite layer, and discloses, as a technique for manufacturing a plated steel sheet, a method of adjustment to an atmosphere containing 2 to 20 vol % of hydrogen and the balance containing nitrogen and impurities and having a dew-point temperature of more than -30° C. and 20° C. or less.

**PATENT LITERATURE**

Patent Literature 1: JP 2011-111670 A

Patent Literature 2: JP 2013-163827 A

Patent Literature 3: JP 2017-048412 A

**Non-Patent Literature**

Non-Patent Literature 1: Kohji Hasegawa, and five others, "980 MPa-kyu Cho-ko-kyodo Kohan no Mage-kako-sei ni Oyobosu Kinzoku-soshiki no Eikyo" (Influence of Metal Structure on the Bending Formability of an Ultrahigh-strength Steel Sheet of the 980-MPa Class), CAMP-ISIJ, vol. 20 (2007), p. 437, published by The Iron and Steel Institute of Japan

Non-Patent Literature 2: Nobuyuki Nakamura, and three others, "Cho-ko-kyodo Reien Kohan no Nobi-furanji-seikei-sei ni Oyobosu Soshiki no Eikyo" (Influence of Structure on the Stretch Flange Moldability of an Ultrahigh-strength Cold Rolled Steel Sheet), CAMP-ISIJ, vol. 13 (2000), p. 391, published by The Iron and Steel Institute of Japan

**SUMMARY OF THE INVENTION**

Thus far, to improve the bendability of a steel sheet, mainly the optimization of steel structure has been made; however, this provides only a certain level of improvement, and further improvement is required. Further, it is presumed that, in the case where a high alloy-based steel sheet is subjected to plating, hydrogen in the atmosphere in the plating step becomes hydrogen in steel remaining in the steel sheet product. It is presumed that improvement in bendability is hindered by the hydrogen in steel. It is also necessary to achieve both improvement in bendability and plating ability.

Aspects of the present invention improve the bendability of a plated steel sheet from a new point of view, and an

object according to aspects of the present invention is to provide a high-strength galvanized steel sheet and a high strength member excellent in plating ability and bendability, and a method for manufacturing them.

The high strength referred to in the present specification means that tensile strength (TS) is 1100 MPa or more.

The present inventors conducted extensive studies in order to solve the issue mentioned above. As a result, it has been found out that, to improve the bendability of a plated steel sheet, it is necessary to appropriately adjust the amount of hydrogen remaining in the steel in addition to the existence state of inclusions existing from the vicinity of the outer layer in the sheet thickness to near the center of the sheet thickness. Further, it has been found out that a high-strength galvanized steel sheet having good bendability and plating ability is obtained by, in addition to controlling inclusions and adjusting the amount of hydrogen in the steel, setting the steel sheet to a specific chemical composition and adjusting particularly the mass ratio of the content of Si to the content of Mn in the steel (Si/Mn) to a predetermined range.

Further, it has been found out that a high-strength galvanized steel sheet according to aspects of the present invention can be manufactured by appropriately adjusting conditions of manufacturing steps, such as conditions of an atmosphere in the furnace during recrystallization annealing. In particular, in the course of studies on manufacturing conditions of a galvanized steel sheet according to aspects of the present invention, the present inventors have found for the first time that the plating ability of the galvanized steel sheet can be dramatically improved by incorporating a specific chemical composition into the steel, setting particularly the mass ratio of the content of Si to the content of Mn in the steel (Si/Mn) to 0.1 or more and less than 0.2, and controlling the dew-point temperature of the atmosphere in the furnace in an annealing step to a specific range. This is presumed to be because, by controlling the dew-point temperature, elements that are likely to be oxidized in the steel have been appropriately controlled in a successful manner and particularly the external oxidation of Mn has been effectively suppressed in a successful manner. Specifically, aspects of the present invention provide the following.

[1] A high-strength galvanized steel sheet including:

a steel sheet having a chemical composition containing a steel composition containing, in mass %,

C: 0.08% or more and 0.20% or less,

Si: less than 2.0%,

Mn: 1.5% or more and 3.5% or less,

P: 0.02% or less,

S: 0.002% or less,

Al: 0.10% or less, and

N: 0.006% or less,

a mass ratio of a content of Si to a content of Mn in the steel (Si/Mn) being 0.1 or more and less than 0.2, and the balance: Fe and incidental impurities, and

a steel structure in which an average grain size of inclusions containing at least one of Al, Si, Mg, and Ca and existing in an area extending from a surface to a position of  $\frac{1}{3}$  of a sheet thickness is 50  $\mu\text{m}$  or less, and an average nearest distance between the inclusions is 20  $\mu\text{m}$  or more; and

a galvanized layer provided on a surface of the steel sheet and having a coating weight per one surface of 20  $\text{g}/\text{m}^2$  or more and 120  $\text{g}/\text{m}^2$  or less,

in which an amount of diffusible hydrogen contained in the steel is less than 0.25 mass ppm, and

a tensile strength is 1100 MPa or more.

[2] The high-strength galvanized steel sheet according to [1], in which the chemical composition further contains, in mass %, at least one of (1) to (3) below,

(1) one or more of Ti, Nb, V, and Zr: 0.005% or more and 0.1% or less in total,

(2) one or more of Mo, Cr, Cu, and Ni: 0.01% or more and 0.5% or less in total, and

(3) B: 0.0003% or more and 0.005% or less.

[3] The high-strength galvanized steel sheet according to 10 any one of [1] or [2], in which the chemical composition further contains, in mass %, at least one of Sb: 0.001% or more and 0.1% or less and Sn: 0.001% or more and 0.1% or less.

[4] The high-strength galvanized steel sheet according to 15 any one of [1] to [3], in which the chemical composition further contains, in mass %, Ca: 0.0005% or less.

[5] The high-strength galvanized steel sheet according to any one of [1] to [4],

in which the steel structure contains 40% or more and 20 90% or less of martensite, 50% or less (including 0%) of ferrite, 50% or less (including 0%) of bainite, and less than 3% (including 0%) of retained austenite in terms of area ratio, and

an average grain size of ferrite is 25  $\mu\text{m}$  or less.

[6] A method for manufacturing a high-strength galvanized steel sheet, including:

a casting step of casting steel having the chemical composition according to any one of [1] to [4] under a condition where a flow velocity of molten steel at a solidification 30 interface in vicinity of a meniscus of a casting mold is 16  $\text{cm}/\text{s}$  or more, and producing a steel raw material;

a hot rolling step of hot rolling the steel raw material after the casting step;

a pickling step of pickling a steel sheet after the hot rolling 35 step;

a cold rolling step of cold rolling the steel sheet after the pickling step at a rolling reduction ratio of 20% or more and 80% or less;

an annealing step of heating the steel sheet after the cold 40 rolling step in a continuous annealing line at an annealing temperature of  $(\text{Ac}3-30)^\circ\text{C}$ . or more and  $(\text{Ac}3+20)^\circ\text{C}$ . or less, with a hydrogen concentration of an atmosphere in the furnace of 500  $^\circ\text{C}$ . or more set to more than 0 vol % and less than 10 vol % and a dew-point temperature of an atmosphere

45 in the furnace of 750  $^\circ\text{C}$ . or more set to  $-45^\circ\text{C}$ . or less, then performing cooling at an average cooling rate of 3  $^\circ\text{C}/\text{s}$  or more from the annealing temperature to at least 600  $^\circ\text{C}$ ., and then performing retaining in a temperature region of 500  $^\circ\text{C}$ . to 400  $^\circ\text{C}$ . for 45 seconds or more; and

50 a plating step of subjecting the steel sheet after the annealing step to plating treatment, and after the plating treatment, performing cooling at an average cooling rate of 3  $^\circ\text{C}/\text{s}$  or more through a temperature region of 450  $^\circ\text{C}$ . to 250  $^\circ\text{C}$ .

55 [7] The method for manufacturing a high-strength galvanized steel sheet according to [6], further including, after the plating step, a width trimming step of performing width trimming.

[8] The method for manufacturing a high-strength galvanized steel sheet according to [6] or [7], further including, after the annealing step or after the plating step, a post-treatment step of performing heating in a temperature region of 50 to 400  $^\circ\text{C}$ . for 30 seconds or more in an atmosphere with a hydrogen concentration of 5 vol % or less and a dew-point temperature of 50  $^\circ\text{C}$ . or less.

[9] The method for manufacturing a high-strength galvanized steel sheet according to any one of [6] to [8], in which

alloying treatment is performed immediately after the plating treatment in the plating step.

[10] A high strength member, obtained by subjecting the high-strength galvanized steel sheet according to any one of [1] to [5] to at least either one of forming and welding.

[11] A method for manufacturing a high strength member, including a step of performing at least either one of forming and welding on a high-strength galvanized steel sheet manufactured by the method for manufacturing a high-strength galvanized steel sheet according to any one of [6] to [9].

According to aspects of the present invention, a high-strength galvanized steel sheet and a high strength member excellent in plating ability and bendability and a method for manufacturing them can be provided. In the case where a high-strength galvanized steel sheet according to aspects of the present invention is used for a framework member of an automobile body, the high-strength galvanized steel sheet can make a great contribution to improvement in collision safety and weight reduction.

#### BRIEF DESCRIPTION OF THE DRAWINGS

The FIGURE is a diagram showing an example of relationship between the amount of diffusible hydrogen in steel and R/t.

#### DETAILED DESCRIPTION OF EMBODIMENTS OF THE INVENTION

Hereafter, the embodiments of the present invention will be described. Here, the present invention is not limited to the embodiments described below.

A high-strength galvanized steel sheet according to aspects of the present invention includes a steel sheet and a galvanized layer formed on a surface of the steel sheet. First, the chemical composition of the steel sheet (a steel composition) will be described. In the description of the chemical composition of the steel sheet, “%” that is the unit of the content of a component means “mass %”.

C: 0.08% or more and 0.20% or less.

C is an effective element to increase the strength of the steel sheet, and contributes to strength increase by forming martensite, which is a hard phase of steel structure. Further, depending on the manufacturing method, C contributes to strength increase also by forming a fine alloy compound or an alloy carbonitride together with a carbide-forming element such as Nb, Ti, V, or Zr. To obtain these effects, the content of C needs to be set to 0.08% or more. On the other hand, if the content of C is more than 0.20%, martensite is hardened excessively, and bending formability tends not to be improved even if inclusions or the amount of hydrogen in the steel is controlled. Thus, the content of C is set to 0.08% or more and 0.20% or less. From the viewpoint of stably achieving a TS of 1100 MPa or more, the content of C is preferably 0.09% or more.

Si: less than 2.0%

Si is an element contributing mainly to strength increase by solid solution strengthening; and experiences relatively small reduction in ductility with respect to strength increase, and contributes to not only strength but also improvement in balance between strength and ductility. Improvement in ductility leads to improvement in bendability. On the other hand, Si is likely to form Si-based oxides on the surface of the steel sheet, and may be a cause of bare spot. Further, in the case where Si coexists with Mn, also the effect of suppressing bare spot is exhibited by causing Si—Mn-based composite oxides to be formed; however, if Si is contained

excessively, significant scales are formed during hot rolling and scale flaws are marked on the surface of the steel sheet, and consequently surface quality may be deteriorated. Thus, it is sufficient to add Si only an amount necessary to ensure strength; from the viewpoint of plating ability, the content of Si is set to less than 2.0%. Further, from the viewpoint of effectively obtaining the effect according to aspects of the present invention by setting the mass ratio of the content of Si to the content of Mn in the steel (Si/Mn) to within the range according to aspects of the present invention, the content of Si is preferably 0.65% or less, and more preferably 0.50% or less. The lower limit of the content of Si is not particularly prescribed; however, if the content of Si is less than 0.001%, control in manufacturing tends to be difficult; thus, the content of Si is preferably set to 0.001% or more. From a viewpoint where it is sufficient to add only an amount necessary to ensure strength, a more preferred content of Si is 0.3% or more.

20 Mn: 1.5% or more and 3.5% or less

Mn is effective as an element contributing to strength increase by solid solution strengthening and martensite formation, and to obtain this effect, the content of Mn needs to be set to 1.5% or more. The content of Mn is preferably 1.9% or more. On the other hand, if the content of Mn is more than 3.5%, unevenness is likely to occur in the steel structure due to segregation or the like of Mn and formability decreases, and Mn is likely to be externally oxidized as oxides or composite oxides on the surface of the steel sheet, and may be a cause of bare spot. Thus, the content of Mn is set to 3.5% or less.

P: 0.02% or less

P is an effective element contributing to the strength increase of the steel sheet by solid solution strengthening, but on the other hand influences plating ability. In particular, P causes degradation in wettability with the steel sheet and reduction in the alloying rate of a coating layer, and there is great influence particularly in a high alloy system whereby a high-strength steel sheet is obtained. Thus, the content of P is set to 0.02% or less. The content of P is preferably 0.01% or less. The lower limit of the content of P is not particularly prescribed; however, if the lower limit is less than 0.0001%, a reduction in production efficiency and deposphorization cost increase are brought about in the manufacturing process; thus, the content of P is preferably set to 0.0001% or more.

S: 0.002% or less

S is likely to form sulfide-based inclusions in the steel. In particular, in the case where a large amount of Mn is added for strength increase, MnS-based inclusions are likely to be formed. This is a cause of impairing bendability; in addition, S causes hot brittleness, and gives adverse effect on the manufacturing process; thus, the amount of S is preferably reduced as much as possible. In accordance with aspects of the present invention, up to 0.002% is acceptable. The lower limit of the content of S is not particularly prescribed; however, if the lower limit is less than 0.0001%, a reduction in production efficiency and cost increase are brought about in the manufacturing process; thus, the content of S is preferably set to 0.0001% or more.

Al: 0.10% or less

Al is added as a deoxidizer. In the case where Al is added as a deoxidizer, it is preferable that 0.001% or more of Al be contained in order to obtain this effect. On the other hand, if the content of Al is more than 0.10%, inclusions are likely

to be formed during the manufacturing process, and bendability is degraded. Thus, the content of Al is set to 0.10% or less, and is preferably 0.08% or less as sol. Al in the steel.

N: 0.006% or less

If the content of N is more than 0.006%, excessive nitrides are produced in the steel and formability is reduced, and the deterioration of the surface quality of the steel sheet may be caused. Hence, the content of N is set to 0.006% or less, and preferably 0.005% or less. If there is ferrite, although the content is preferably as small as possible from the viewpoint of improving ductility by refining ferrite, such amounts reduce production efficiency and increase cost in the manufacturing process; thus, the content of N is preferably set to 0.0001% or more.

A mass ratio of a content of Si to a content of Mn in the steel (Si/Mn) is 0.1 or more and less than 0.2

To obtain more excellent plating ability, it is important to control elements that are likely to be oxidized in the steel. In the case where it is assumed that the manufacturing method described below is used, the mass ratio of the content of Si to the content of Mn in the steel (Si/Mn) needs to be 0.1 or more in order to produce Si—Mn composite oxides from the viewpoint of suppressing the external oxidation of Mn. If the mass ratio (Si/Mn) is 0.2 or more, oxides of mainly Si are likely to be formed, and this is a factor of bare spot; thus, the mass ratio (Si/Mn) is set to less than 0.2. In the case where it is assumed that the manufacturing method described below is used, the mass ratio of the content of Si to the content of Mn in the steel (Si/Mn) is preferably set to 0.11 or more and less than 0.19 from the viewpoint of obtaining excellent plating ability.

The steel according to aspects of the present invention basically contains the chemical composition mentioned above, and the balance is iron and incidental impurities. In the chemical composition mentioned above, the components mentioned below may be further contained as arbitrary components to the extent that the action according to aspects of the present invention is not impaired. In the case where any of the arbitrary elements mentioned below is contained at less than the lower limit value mentioned below, it is assumed that the arbitrary component is contained as an incidental impurity. Further, in the chemical composition, Mg, La, Ce, Bi, W, and Pb may be contained as incidental impurities up to 0.002% in total.

The chemical composition mentioned above may further contain, as arbitrary components, at least one of (1) to (3) below in mass %.

(1) one or more of Ti, Nb, V, and Zr: 0.005% or more and 0.1% or less in total,

(2) one or more of Mo, Cr, Cu, and Ni: 0.01% or more and 0.5% or less in total, and

(3) B: 0.0003% or more and 0.005% or less.

Ti, Nb, V, and Zr form, together with C or N, carbides or nitrides (also possibly carbonitrides). These elements contribute to the strength increase of the steel sheet by being formed in fine precipitates. In particular, by precipitating these elements in soft ferrite, the strength of the soft ferrite is enhanced, and the strength difference with martensite is reduced; this effect contributes to improvement in not only bendability but also stretch flangeability. Further, these elements have the action of refining the structure of a hot rolled coil; thus, contribute to strength increase and improvement in formability such as bendability also by refining the steel structure after cold rolling and annealing subsequent to the hot rolling. From the viewpoint of obtaining this effect, it is preferable that one or more of Ti, Nb, V, and Zr be contained at 0.005% or more in total. However,

excessive addition increases deformation resistance during cold rolling and inhibits productivity, and the presence of excessive or coarse precipitates tends to reduce the ductility of ferrite and reduce the ductility or bendability of the steel sheet. Hence, it is preferable that one or more of Ti, Nb, V, and Zr be contained 0.1% or less in total.

The elements of Mo, Cr, Cu, and Ni enhance hardenability and facilitate generation of martensite, and are therefore elements contributing to strength increase. To obtain these effects, the lower limit mentioned above of 0.01% is prescribed as a preferred lower limit. Excessive addition of Mo, Cr, Cu, and Ni leads to the saturation of the effect and cost increase; further, Cu induces cracking during hot rolling, and is a cause of the occurrence of surface flaws. Thus, it is preferable that one or more of Mo, Cr, Cu, and Ni be contained 0.5% or less in total. Ni has the effect of impeding the occurrence of surface flaws resulting from Cu addition, and is therefore preferably added in a simultaneous manner when Cu is added. In particular, the content of Ni is preferably  $\frac{1}{2}$  or more of the amount of Cu.

Also for B, in addition to the lower limit mentioned above for obtaining the effect of suppressing ferrite formation occurring during an annealing cooling process, an upper limit is provided for the excessive addition due to the saturation of the effect. Excessive hardenability has also a disadvantage such as weld cracking during welding. Thus, the content of B is preferably set to 0.0003% or more and 0.005% or less.

The chemical composition mentioned above may further contain, as an optional component, the following component.

At least one of Sb: 0.001% or more and 0.1% or less and Sn: 0.001% or more and 0.1% or less

Sb and Sn are effective elements to suppress decarburization, denitridification, deboronization, etc., and suppress the strength reduction of the steel sheet; thus, the content of each element is preferably 0.001% or more. However, excessive addition reduces surface quality; thus, the upper limit of the content of each element is preferably set to 0.1%.

Ca: 0.0005% or less

When a small amount of Ca is added, the effect of spheroidizing the shapes of sulfides and improving the bendability of the steel sheet is obtained. On the other hand, if Ca is added excessively, Ca forms sulfides or oxides in the steel excessively, and reduces the formability, particularly bendability, of the steel sheet; thus, the content of Ca is preferably set to 0.0005% or less. The lower limit of the content of Ca is not particularly prescribed; however, in the case where Ca is contained, the content of Ca is often 0.0001% or more.

Next, the steel structure of the steel sheet is described.

In the steel structure, the average grain size of inclusions containing at least one of Al, Si, Mg, and Ca and existing in an area extending from a surface to a position of  $\frac{1}{3}$  of the sheet thickness is 50  $\mu\text{m}$  or less, and the average nearest distance between inclusions is 20  $\mu\text{m}$  or more. Bendability can be improved when the average grain size of inclusions and the average nearest distance between inclusions are adjusted to the ranges mentioned above and the amount of diffusible hydrogen in the steel is set in a specific range. In the measurement of the nearest distance between inclusions, inclusions other than inclusions containing at least one of Al, Si, Mg, and Ca are not included.

The average grain size of inclusions is 50  $\mu\text{m}$  or less, preferably 30  $\mu\text{m}$  or less, and more preferably 20  $\mu\text{m}$  or less.

The average grain size of inclusions is preferably as small as possible; thus, the lower limit is not particularly prescribed, but is often 1  $\mu\text{m}$  or more.

The average nearest distance of inclusions is 20  $\mu\text{m}$  or more, preferably 30  $\mu\text{m}$  or more, and more preferably 50  $\mu\text{m}$  or more. As for the average nearest distance of inclusions, the upper limit is not particularly prescribed, but is often 500  $\mu\text{m}$  or less.

The average grain size of inclusions and the average nearest distance between inclusions are measured by methods described in Examples.

Further, in accordance with aspects of the present invention, the steel structure of a steel sheet preferably contains 40% or more and 90% or less of martensite, 50% or less (including 0%) of ferrite, 50% or less (including 0%) of bainite, and less than 3% (including 0%) of retained austenite in terms of area ratio, and an average grain size of ferrite is 25  $\mu\text{m}$  or less.

#### Martensite: 40% or more and 90% or less

Martensite is a hard structure, and is effective and essential to enhance the strength of the steel sheet. In order to ensure a tensile strength (TS) of 1100 MPa or more, the amount of martensite is preferably set to 40% or more in terms of area ratio. From the viewpoint of ensuring TS stably, the amount of martensite is preferably set to 45% or more. The martensite herein includes autotempered martensite that is self-tempered during manufacturing and, depending on the circumstances, tempered martensite that is tempered by a subsequent heat treatment. From the viewpoint of the balance between bendability and strength, the amount of martensite is preferably set to 90% or less.

#### Ferrite: 50% or less (including 0%)

In the case where heat treatment and a step of providing plating are performed in an atmosphere where hydrogen exists, hydrogen enters the interior of the steel and remains in the steel. As a technique for reducing the amount of hydrogen in the steel of the end product as much as possible, ferrite and bainite having BCC structures are formed in the steel structure before providing plating. This utilizes the fact that the solid solubility of hydrogen is smaller in ferrite and bainite having BCC structures than in austenite having an FCC structure. Further, soft ferrite improves the ductility of the steel sheet, and improves bendability. However, if ferrite exceeds 50%, strength cannot be ensured; thus, a preferred upper limit is set to 50%. Ferrite often accounts for 2% or more.

The average grain size of ferrite is preferably 25  $\mu\text{m}$  or less. The smaller the ferrite grain size is, the more the generation and linkage of voids on the bending surface can be suppressed, and the more the bendability can be enhanced. The average grain size of ferrite is more preferably 20  $\mu\text{m}$  or less, and still more preferably 15  $\mu\text{m}$  or less.

#### Bainite: 50% or less (including 0%)

Bainite contributes to improvement in bendability, and may therefore be contained; however, if bainite is contained excessively, desired strength is not obtained and bendability is degraded; thus, the amount of bainite is preferably set to 50% or less. Bainite often accounts for 2% or more.

Retained austenite accounting for less than 3% (including 0%)

Austenite is an fcc phase; as compared to ferrite (a bcc phase), austenite has high ability of occluding hydrogen, and is diffused slowly in the steel and is therefore likely to remain in the steel. Further, in the case where the retained austenite experiences strain-induced transformation to martensite, there is a concern that the amount of diffusible hydrogen in the steel will be increased. Thus, in accordance

with aspects of the present invention, retained austenite preferably accounts for less than 3%.

The steel structure occasionally contains precipitates of pearlite, carbides, etc. in the balance, as structures other than the structures (phases) mentioned above; these can be permitted as long as they account for 10% or less as the total area ratio in a position of  $1/4$  of the sheet thickness from the surface of the steel sheet. The amount of these other structures is preferably set to 5% or less (including 0%).

The inclusions and the area ratios of the steel structure mentioned above are found by methods described in Examples.

Next, the galvanized layer is described. For the galvanized layer, the coating weight per one surface is 20 to 120  $\text{g}/\text{m}^2$ . If the coating weight is less than 20  $\text{g}/\text{m}^2$ , it is difficult to ensure corrosion resistance. Thus, the coating weight is set to 20  $\text{g}/\text{m}^2$  or more, preferably 25  $\text{g}/\text{m}^2$  or more, and more preferably 30  $\text{g}/\text{m}^2$  or more. On the other hand, if the coating weight is more than 120  $\text{g}/\text{m}^2$ , plating peeling resistance is degraded. Thus, the coating weight is 120  $\text{g}/\text{m}^2$  or less, preferably 100  $\text{g}/\text{m}^2$  or less, and more preferably 80  $\text{g}/\text{m}^2$  or less.

The composition of the galvanized layer is not particularly limited, and may be a common composition. For example, in the case of a hot-dip galvanized layer or an alloyed hot-dip galvanized layer, the composition is generally a composition containing Fe: 20 mass % or less and Al: 0.001 mass % or more and 1.0 mass % or less, further containing one or two or more selected from Pb, Sb, Si, Sn, Mg, Mn, Ni, Cr, Co, Ca, Cu, Li, Ti, Be, Bi, and REMs at 0 mass % or more and 3.5 mass % or less in total, and containing the balance containing Zn and incidental impurities. In accordance with aspects of the present invention, it is preferable to have a hot-dip galvanized layer in which the coating weight per one surface is 20 to 120  $\text{g}/\text{m}^2$  or an alloyed hot-dip galvanized layer in which the hot-dip galvanized layer is further alloyed. In the case where the coating layer is a hot-dip galvanized layer, the content of Fe in the coating layer is preferably less than 7 mass %; in the case where the coating layer is an alloyed hot-dip galvanized layer, the content of Fe in the coating layer is preferably 7 to 20 mass %.

In the high-strength galvanized steel sheet according to aspects of the present invention, the amount of diffusible hydrogen in the steel obtained by measurement by a method described in Examples is less than 0.25 mass ppm. Diffusible hydrogen in the steel degrades bendability. If the amount of diffusible hydrogen in the steel is 0.25 mass ppm or more, bendability is deteriorated even if inclusions and steel structure are produced properly.

In accordance with aspects of the present invention, it has been revealed that a stable improvement effect is provided by setting the amount of diffusible hydrogen in the steel to less than 0.25 mass ppm. The amount of diffusible hydrogen in the steel is preferably 0.20 mass ppm or less, and more preferably 0.15 mass ppm or less. The lower limit is not particularly limited, but is preferably as small as possible; thus, the lower limit is 0 mass ppm. In accordance with aspects of the present invention, it is necessary that, before subjecting the steel sheet to forming or welding, diffusible hydrogen in the steel accounts for less than 0.25 mass ppm. Note that, if the amount of diffusible hydrogen in the steel measured by using a sample cut out from a product (a member) that is obtained after subjecting the steel sheet to forming or welding and that is placed in a common usage environment is less than 0.25 mass ppm, the amount of

## 11

diffusible hydrogen in the steel can be regarded as having been less than 0.25 mass ppm also before the forming or the welding.

The high-strength galvanized steel sheet according to aspects of the present invention has high tensile strength (TS). Specifically, the tensile strength (TS) measured by a method described in Examples is 1100 MPa or more. The sheet thickness of the high-strength galvanized steel sheet according to aspects of the present invention is not particularly limited, but is preferably set to 0.5 mm or more and 3 mm or less.

Next, a method for manufacturing a high-strength galvanized steel sheet according to aspects of the present invention is described. The manufacturing method according to aspects of the present invention includes a casting step, a hot rolling step, a pickling step, a cold rolling step, an annealing step, and a plating step. Each step will now be described. The temperatures at the time of heating or cooling slabs (steel raw materials), steel sheets, etc. shown below mean, unless otherwise stated, the surface temperatures of the slabs (the steel raw materials), the steel sheets, etc.

The casting step is a step of casting steel having the chemical composition mentioned above under a condition where the flow velocity of molten steel at the solidification interface in the vicinity of the meniscus of the casting mold is 16 cm/s or more, and producing a steel raw material.

## Manufacturing of Steel Raw Material (Slab (Cast Piece))

As the steel used in the manufacturing method according to aspects of the present invention, steel manufactured by a continuous casting method, generally called a slab, is used; this is for the purpose of preventing macro-segregation of alloy components; the manufacturing may be performed also by an ingot casting, a thin slab casting method, or the like.

In the case where continuous casting is performed, casting is performed under a condition where the flow velocity of molten steel at the solidification interface in the vicinity of the meniscus of the casting mold (hereinafter, also referred to simply as the flow velocity of molten steel) is 16 cm/s or more, from the viewpoint of controlling inclusions. The flow velocity of molten steel is preferably 17 cm/s or more. By increasing the flow velocity of molten steel, it becomes easy to obtain a steel sheet according to aspects of the present invention; thus, the upper limit is not particularly prescribed; however, from the viewpoint of operating stability, the upper limit is preferably set to 50 cm/s or less. "The vicinity of the meniscus of the casting mold" means the interface between powder used during continuous casting and molten steel in the casting mold. In the case of ingot making, it is preferable that inclusions be caused to sufficiently float up during solidification, the place where the inclusions float up and gather be cut off, and the resulting piece be used for the next step.

A hot rolling step is a step of hot rolling the steel raw material after the casting step

After a steel slab has been manufactured, hot rolling may be performed by using any one of a conventional method in which the slab is reheated after having been cooled to room temperature, a method in which hot rolling is performed after the slab has been charged into a reheating furnace in the warm state without having been cooled to near-room temperature, a method in which hot rolling is performed immediately after the slab has been subjected to heat retention for a short time, and a method in which hot rolling is performed directly on a cast piece in the hot state without problem.

The method of hot rolling is not particularly prescribed, but is preferably performed under the following conditions.

## 12

It is preferable that the steel slab reheating temperature be 1100° C. or more and 1350° C. or less. The grain diameter of precipitates in the steel slab tends to increase, and there is a disadvantage in that it is difficult, for example, to achieve satisfactory strength through precipitation strengthening. Because there may be a case where precipitates having a large grain diameter have negative effects on the formation of a microstructure in the subsequent annealing process. Further, achieving a smooth steel sheet surface by heating in order to remove, for example, blowholes and defects from the surface of the slab through scale off so that there is a decrease in the number of cracks and in the degree of asperity on the surface of a steel sheet is advantageous as product quality. From this viewpoint, the slab reheating temperature is prescribed. It is preferable that the reheating temperature be 1100° C. or more in order to realize such an effect. On the other hand, in the case where the reheating temperature is more than 1350° C., since there is an increase in austenite grain diameter, there is an increase in the grain diameter of the steel structure of an end product, which may result in a deterioration in the strength and bendability of a steel sheet, therefore, the preferable upper limit is prescribed.

In the hot rolling step including rough rolling and finish rolling, generally, a steel slab is made into a sheet bar by performing rough rolling, and the sheet bar is made into a hot-rolled coil by performing finish rolling, however, there is no problem in the case where rolling is performed regardless of such a classification depending on, for example, rolling mill capacity as long as a predetermined size is obtained.

The following are recommended as hot rolling conditions.

The finishing delivery temperature is preferably set in the range of 800° C. or more and 950° C. or less. This is aimed at, by the setting to 800° C. or more, making uniform the structure obtained in the hot rolled coil and allowing also the structure of the end product to be uniform. If the structure is non-uniform, bendability tends to be reduced. On the other hand, in the case where the finishing delivery temperature is more than 950° C., since there is an increase in the amount of oxides (scale) formed, there is an increase in the degree of asperity of an interface between the base steel and the oxides, which may tend to result in a deterioration in the surface quality after pickling or cold rolling. Further, the crystal grain size is increased, and this tends to be a cause of reducing the strength and the bendability of the steel sheet, like in a steel slab.

The hot rolled coil (hot rolled sheet) after completion of the hot rolling as described above is, for the purpose of the refinement and homogenization of a microstructure, preferably started to be cooled within 3 seconds after finish rolling has been performed at an average cooling rate of 10 to 250° C./s in a temperature region from [finishing delivery temperature] to [finishing delivery temperature-100]° C., and cooled in a temperature region from 450 to 700° C.

The pickling step is a step of pickling the steel sheet after the hot rolling step. Scales are dropped by pickling. Pickling conditions may be set as appropriate.

The cold rolling step is a step of cold rolling the steel sheet after the pickling step at a rolling reduction ratio of 20% or more and 80% or less.

The reason why the rolling reduction ratio is set to 20% or more is that it is attempted to obtain uniform fine steel structure in the annealing step subsequently performed. If the rolling reduction ratio is less than 20%, it is likely that coarse grains will be produced and non-uniform structure will be produced during annealing, and it is feared that

strength and formability in the end product sheet will be reduced as described above. For the upper limit, a high rolling reduction ratio may cause not only reduction in productivity due to the rolling load but also shape failure; thus, the upper limit is set to 80%. It is also possible to perform pickling after cold rolling.

An annealing step is a step of heating the steel sheet after the cold rolling step in a continuous annealing line at an annealing temperature of  $(Ac3-30)^\circ C.$  or more and  $(Ac3+20)^\circ C.$  or less in an atmosphere in the furnace in which a hydrogen concentration of  $500^\circ C.$  or more is more than 0 vol % and less than 10 vol % and a dew-point temperature in the atmosphere in the furnace of  $750^\circ C.$  or more is  $-45^\circ C.$  or less, then performing cooling at an average cooling rate of  $3^\circ C./s$  or more from the annealing temperature to at least  $600^\circ C.$ , and then performing retaining in a temperature region of  $500^\circ C.$  to  $400^\circ C.$  for 45 seconds or more. The cooling stop temperature of cooling is not particularly limited. The  $Ac3$  transformation point (in the present specification, also written as simply  $Ac3$ ) is calculated in the following way.

$$Ac3(\text{° C.}) = 910 - 203(C)_{1/2} + 44.7\text{Si} - 30\text{Mn} - 11\text{P} + 700\text{S} + 400\text{A1} + 400\text{Ti}$$

The atomic symbols in the equations above respectively denote the contents of the corresponding chemical elements, and where the symbol of a chemical element which is not contained is assigned a value of 0.

If the hydrogen concentration of the atmosphere in the furnace of  $500^\circ C.$  or more is too high, there is a problem that the amount of diffusible hydrogen in the steel prescribed in accordance with aspects of the present invention becomes more than the upper limit; if the annealing temperature is too low, there is a problem of poor plating ability; thus, the hydrogen concentration of the atmosphere in the furnace of  $500^\circ C.$  or more is set to more than 0 vol % and less than 10 vol %. The hydrogen concentration is preferably 8 vol % or less. From the viewpoint of improving plating ability, the hydrogen concentration is preferably 1 vol % or more, and more preferably 3 vol % or more.

In the case where the dew-point temperature of an atmosphere in the furnace of  $750^\circ C.$  or more is more than  $-45^\circ C.$ , in the present component system, the external oxidation of oxides containing Si and Mn cannot be suppressed, and bare spot is caused. Hence, the dew-point temperature is set to  $-45^\circ C.$  or less. For an atmosphere of less than  $750^\circ C.$ , the influence on the external oxidation of oxides containing Si and Mn is small, and hence the dew-point temperature is not particularly prescribed; however, from the viewpoint of ensuring the airtightness of the furnace body, the dew-point temperature is preferably  $-55^\circ C.$  or more and  $10^\circ C.$  or less in view of the fact that it is very difficult to maintain a dew-point temperature of  $-55^\circ C.$  or less and that dew-point temperatures of  $10^\circ C.$  or more have the concern of the degradation of the roll due to pickup, etc.

If the annealing temperature is too high, there is a problem that the amount of diffusible hydrogen in the steel prescribed in accordance with aspects of the present invention exceeds the upper limit; if the annealing temperature is too low, there is a problem that the microstructure and the tensile strength prescribed in accordance with aspects of the present invention are not obtained; thus, the annealing temperature is set to  $(Ac3-30)^\circ C.$  or more and  $(Ac3+20)^\circ C.$  or less.

If the average cooling rate from the annealing temperature to at least  $600^\circ C.$  is too slow, there is a problem that an amount of martensite for obtaining desired characteristics cannot be ensured; thus, the average cooling rate is set to  $3^\circ$

$C./s$  or more. The average cooling rate from the annealing temperature to at least  $600^\circ C.$  is preferably  $4^\circ C./s$  or more. The reason for focusing on the temperature region of the annealing temperature to at least  $600^\circ C.$  is that this temperature region is a temperature region that easily forms ferrite and pearlite structure and influences the amount of austenite to become martensite. The upper limit of the average cooling rate from the annealing temperature to at least  $600^\circ C.$  is not particularly prescribed; however, from the viewpoint of energy saving of the cooling facility, the upper limit is preferably set to  $200^\circ C./s$  or less.

Cooling is performed at an average cooling rate of  $3^\circ C./s$  or more from the annealing temperature to at least  $600^\circ C.$ , and then the steel sheet is retained in the temperature region of  $500^\circ C.$  to  $400^\circ C.$  for 45 seconds or more. Thereby, the effect of suppressing the variation in the temperature of a plating bath is obtained in the plating step performed next. If the retention time is set long, the amount of bainite structure tends to be increased. Here, the temperature may be brought within the temperature region of  $500$  to  $400^\circ C.$  by performing cooling from the annealing temperature to at least  $600^\circ C.$  and then performing cooling continuously, or may be brought within the temperature region of  $500$  to  $400^\circ C.$  by temporarily performing cooling up to a temperature lower than  $400^\circ C.$  and then performing reheating. In the case of the latter, when cooling is temporarily performed up to the  $Ms$  point or less, tempering may be performed after martensite is generated.

The plating step is a step of subjecting the steel sheet after the annealing step to plating treatment and after the plating treatment, performing cooling at an average cooling rate of  $3^\circ C./s$  or more through the temperature region of  $450^\circ C.$  to  $250^\circ C.$

If the average cooling rate in the temperature region of  $450^\circ C.$  to  $250^\circ C.$  after plating treatment is too slow, there is a problem that an amount of martensite necessary to obtain the effect according to aspects of the present invention is less likely to be generated; thus, the average cooling rate is set to  $3^\circ C./s$  or more. The average cooling rate from  $450^\circ C.$  to  $250^\circ C.$  after plating treatment is preferably  $5^\circ C./s$  or more. The reason for focusing on the temperature region of  $450$  to  $250^\circ C.$  is that the temperatures from the plating temperature and/or the plating alloying temperature to the martensite transformation start temperature (the  $Ms$  point) are taken into consideration. The upper limit of the average cooling rate of the region from  $450^\circ C.$  to  $250^\circ C.$  after plating treatment is not particularly prescribed; however, from the viewpoint of energy saving of the cooling facility, the upper limit is preferably set to  $2000^\circ C./s$  or less.

Galvanization is performed by, for example, immersion in a hot-dip galvanization bath. Hot-dip galvanization treatment may be performed by a usual method, and adjustment is made so that the coating weight per one surface is in the range mentioned above.

Alloying treatment of galvanization may be performed immediately after galvanization treatment, as necessary. In this case, the steel sheet is held in the temperature region of  $480$  to  $580^\circ C.$  for approximately 1 to 60 seconds.

From the viewpoint of reducing the amount of diffusible hydrogen, it is preferable to further include, after the annealing step or after the plating step, a post-treatment step of performing heating in a temperature region of  $50$  to  $400^\circ C.$  for 30 seconds or more in an atmosphere with a hydrogen concentration of 5 vol % or less and a dew-point temperature of  $50^\circ C.$  or less. The post-treatment step is preferably performed as the next step after the annealing step or the plating step.

If the hydrogen concentration and the dew-point temperature of the post-treatment step are too high, conversely there is a concern that hydrogen will be likely to enter the interior of the steel and the amount of diffusible hydrogen in the steel prescribed in accordance with aspects of the present invention will be more than the upper limit; thus, it is preferable to create an atmosphere with a hydrogen concentration of 5 vol % or less and a dew-point temperature of 50° C. or less.

If the heating time in the temperature region of 50 to 400° C. is short, the effect of reducing the amount of diffusible hydrogen in the steel is small, and the present step produces only an increase in the number of steps; thus, the heating time in the temperature region of 50 to 400° C. is preferably set to 30 seconds or more. The reason for focusing on the temperature region of 50 to 400° C. is that it is presumed that, in this temperature region, dehydrogenation reaction progresses more than the entry of hydrogen and that, at this temperature or more, there is a concern that material quality and the properties of the coating layer will be degraded.

After the plating step, a width trimming step of performing width trimming may be further included. In the width trimming step, an end portion in the sheet width direction of the steel sheet is sheared. This provides the effect of not only adjusting the width of the product but also reducing the amount of diffusible hydrogen in the steel by diffusible hydrogen being removed from the shear end surface.

The manufacturing of a high-strength galvanized steel sheet according to aspects of the present invention may be performed in a continuous annealing line, or may be performed off-line.

<High Strength Member and Method for Manufacturing Same>

A high strength member according to aspects of the present invention is a member obtained by subjecting a high-strength galvanized steel sheet according to aspects of the present invention to at least either one of forming and welding. A method for manufacturing a high strength member according to aspects of the present invention includes a step of performing at least either one of forming and welding on a high-strength galvanized steel sheet manufactured by a method for manufacturing a high-strength galvanized steel sheet according to aspects of the present invention.

The high strength member according to aspects of the present invention is excellent in bendability; thus, can suppress cracking after bending, and has high reliability in terms of structure as a member. Further, the high strength member is excellent in plating ability, particularly plating peeling resistance. Hence, for example, at the time of press forming a steel sheet into a member, the adhesion of zinc powder or the like to the press mold due to peeling of the galvanized layer can be suppressed, and the occurrence of surface defects of the steel sheet resulting from the adhesion can be suppressed. Thus, the high strength member according to aspects of the present invention has the effect of high productivity during press forming.

As the forming, common processing methods such as press forming may be used without limitations. As the welding, common welding such as spot welding or arc welding may be used without limitations. The high strength member according to aspects of the present invention can be suitably used for, for example, automotive parts.

## EXAMPLES

### Example 1

The studies shown in Example 1 were performed in order to find the influence of the amount of hydrogen in steel.

Molten steel of the chemical composition shown in Table 1 was smelted with a converter, and was made into a slab

under the conditions of a flow velocity of molten steel at the solidification interface in the vicinity of the meniscus of the casting mold of 18 cm/s on average and an average casting rate of 1.8 m/min. The slab was heated to 1200° C., and was 5 made into a hot rolled coil under the conditions of a finish rolling temperature of 840° C. and a coiling temperature of 550° C. Hot rolled steel sheets obtained from the hot rolled coil were pickled, and were then made into cold rolled steel sheets each with a sheet thickness of 1.4 mm under the 10 condition of a cold rolling reduction ratio of 50%. The cold rolled steel sheets were heated to 790° C. (within the range of the Ac3 point+20° C. or less) that is an annealing temperature by annealing treatment in atmospheres in the annealing furnace with various hydrogen concentrations and 15 a dew-point temperature of -30° C., were cooled up to 520° C. at an average cooling rate from the annealing temperature up to 600° C. of 3° C./s, were allowed to stay for 50 seconds, 20 were then galvanized and subjected to alloying treatment, and were cooled from 450° C. to 250° C. at an average cooling rate of 6° C./s; thus, high-strength alloyed galvanized steel sheets (product sheets) were manufactured.

A sample was cut out from each sheet, and hydrogen (the amount of diffusible hydrogen) in the steel was analyzed and 25 bendability was evaluated. The results are shown in the FIGURE.

### Amount of Hydrogen in Steel (Amount of Diffusible Hydrogen)

The amount of hydrogen in the steel was measured by the 30 following method. First, an approximately 5×30-mm test piece was cut out from the plated steel sheet, and then a router (precision grinder) was used to remove the plating on a surface of the test piece, and the test piece was put into a 35 quartz tube. Next, the interior of the quartz tube was substituted with Ar, then the temperature was raised at 200° C./hr, and hydrogen generated until reaching 400° C. was analyzed with a gas chromatograph. In this way, the amount of hydrogen released was measured by the programmed 40 temperature analysis method. The cumulative value of the amount of hydrogen detected in the temperature region of room temperature (25° C.) to less than 210° C. was taken as the amount of diffusible hydrogen in steel.

### Bendability

A 25×100-mm strip test piece was cut out from each of the 45 manufactured plated steel sheets in such a manner that a direction parallel to the rolling direction corresponded to the short side. Next, a 90° V-bending test was performed such that the rolling direction corresponded to a ridge to be 50 formed by bending. Striking that makes pressing against a die with a load of 10 tons for 5 seconds, with the speed of the stroke set to 50 mm/min, was performed. A test was 55 performed by variously changing the curvature radius R of the tip of a V-shaped punch in units of 0.5 steps, and the vicinity of the ridge of the test piece was observed with a lens with a magnifying power of 20 to check the presence or absence of a crack (cracking). R/t was calculated from the smallest curvature radius R among those at which a crack did not occur and the sheet thickness of the test piece (t 60 (mm); the value up to the one hundredths place calculated by rounding up if the one thousandths place was 5 or more and rounding down if it was 4 or less was used), and the resulting R/t was taken as an index of bendability. The smaller the value of R/t is, the better the bendability is.

65 It has been shown that, when the amount of diffusible hydrogen in the steel is less than 0.25 mass ppm, bendability (R/t) is stabilized and is excellent. The conditions of inclu-

sions, etc. of these excellent samples were within the ranges according to aspects of the present invention.

ing an L-cross section (thickness cross section parallel to the rolling direction), by etching the polished cross section

TABLE 1

| Steel No. | Chemical composition (mass %) |      |      |       |        |        |       |       |       |        | Ac3 (° C.) | Si/Mn (Mass ratio) |      |
|-----------|-------------------------------|------|------|-------|--------|--------|-------|-------|-------|--------|------------|--------------------|------|
|           | C                             | Si   | Mn   | P     | S      | N      | Al    | Ti    | Nb    | B      |            |                    |      |
| A         | 0.123                         | 0.30 | 2.65 | 0.008 | 0.0008 | 0.0035 | 0.040 | 0.022 | 0.024 | 0.0020 | 0.0003     | 798                | 0.11 |

### Example 2

In Example 2, galvanized steel sheets shown below were manufactured and evaluated.

Various kinds of molten steel of the chemical compositions shown in Table 2 were smelted with a converter, and were cast to produce slabs under the conditions shown in Table 3; each slab was reheated to 1200° C. and was hot rolled at a finish temperature of 800 to 830° C., and a hot rolled coil was manufactured under the condition of a coiling temperature of 560° C. A hot rolled steel sheet obtained from the hot rolled coil was pickled, was subjected to the steps of cold rolling, annealing, plating treatment, width trimming, and post-treatment under the conditions shown in Table 3; thus, a 1.4-mm-thick galvanized steel sheet was manufactured. Alloying treatment of galvanization was performed immediately after plating treatment (galvanization treatment) under conditions of 500° C. and 20 seconds. The steps of width trimming and post-treatment were performed only in part of the manufacturing conditions.

A sample was extracted from the plated steel sheet obtained in the above manner, structure observation and a tensile test were performed by the methods mentioned below, and the tensile strength (TS), the amount of hydrogen in the steel (the amount of diffusible hydrogen), bendability, and the fractions of steel structures were evaluated and measured. Further, plating ability was evaluated. The evaluation method is as follows.

For manufacturing conditions No. 1 of Table 3, also a galvanized steel sheet was manufactured under the same manufacturing conditions except that alloying treatment of galvanized layer was not performed. As described later, the plating ability of this galvanized steel sheet was evaluated by the presence or absence of a bare spot defect.

#### (1) Tensile Test

A tensile test was performed with a constant tensile speed (crosshead speed) of 10 mm/min on a JIS No. 5 tensile test piece (JIS Z 2201) taken from the steel sheet in a direction perpendicular to the rolling direction. The tensile strength was defined as the maximum load in the tensile test divided by the initial cross-sectional area of the parallel part of the test piece. When the cross-sectional area of the parallel part was calculated, the thickness was defined as the thickness including that of the coating layer.

#### (2) Amount of In-Steel Hydrogen (Amount of Diffusible Hydrogen)

The measurement was performed by a similar method to Example 1.

#### (3) Bendability

The measurement was performed by a similar method to Example 1. In this evaluation,  $R/t \leq 3.5$  was evaluated as excellent in bendability.

#### (4) Microstructure Observation

By taking a sample for microstructure observation from the manufactured hot-dip galvanized steel sheet, by polish-

through the use of a nital solution, by performing observation through the use of a SEM at a magnification of 1500 times in 3 or more fields of view in the etched cross section in order to obtain image data, and by performing image analysis on the obtained image data, area ratio was determined for each of the observed fields of view, and average value of the determined area ratios was calculated. The observation position was set in the vicinity of a position located  $\frac{1}{4}$  of a sheet thickness from the surface thickness. However, the volume ratio of retained austenite (the volume ratio is regarded as the area ratio) was quantified by the intensity of X-ray diffraction; therefore, there is a case of a result in which the sum total of the structures is more than 100%. F of Table 4 stands for ferrite, M for martensite (including tempered martensite), B for bainite, and Residual y for retained austenite. The average grain size of ferrite was found by observing 10 grains by SEM, finding the area ratio of each grain, calculating the circle-equivalent diameter, and averaging the circle-equivalent diameters.

In the structure observation mentioned above, pearlite and aggregations of precipitates and inclusions were observed as other phases in some examples.

#### (5) Inclusion Observation

A ridge portion of the test piece subjected to the 90° V-bending test was forcibly broken, and a cross section of the steel sheet was observed by SEM. The compositions of inclusions existing in an outer layer of the test piece, that is, existing from the surface on the outside of bending to a position of  $\frac{1}{3}$  of the sheet thickness were found by qualitative analysis based on EDX, and oxides containing at least one or more of Al, Si, Mg, and Ca were identified; then, the longest diameter (the dimension of the portion with the longest grain width) of each of the inclusions in an image was measured, the longest diameter was regarded as the grain size, and the average grain size of the inclusions was found. Further, in the field of view, the distance (the nearest distance) from any inclusion existing in an area extending from the surface to a position of  $\frac{1}{3}$  of the sheet thickness to an inclusion located nearest to the inclusion was found, the distance mentioned above was calculated for all the inclusions, and the resulting distances were averaged; thus, the average nearest distance was found.

#### (6) Plating Ability

The surface quality (external appearance) of the manufactured hot-dip galvanized steel sheet was visually observed, and the presence or absence of a bare spot defect was investigated. The term "bare spots" denotes areas having a size of about several micrometers to several millimeters in which no coating layer exists so that the steel sheet is exposed.

Further, the plating peeling resistance (adhesiveness) of the manufactured hot-dip galvanized steel sheet was investigated. In the present Example, a cellophane tape was pressed against a processed portion of the hot-dip galvanized steel sheet where bending of 90° was performed, peeled substances were transferred to the cellophane tape, and the

# US 11,560,614 B2

19

amount of peeled substances on the cellophane tape was found as the counted number of Zn pieces by the X-ray fluorescence method. As measurement conditions, a diameter of a mask of 30 mm, and an accelerating voltage of 50 kV, an accelerating current of 50 mA, and a measuring time of 20 seconds for X-ray fluorescence were used.

Plating ability was evaluated by the following criteria. The results are shown in Table 4. In accordance with aspects of the present invention, rank A, B, or C mentioned below, which has no bare spot defect, was classified as passed.

A: There is no bare spot defect, and the counted number of Zn pieces is less than 7000.

B: There is no bare spot defect, and the counted number of Zn pieces is 7000 or more and less than 8000.

20

C: There is no bare spot defect, and the counted number of Zn pieces is 8000 or more.

D: A bare spot defect occurs.

The plating ability of the galvanized steel sheet not subjected to alloying treatment described above was evaluated by checking the presence or absence of a bare spot defect. Specifically, the surface quality (external appearance) of the galvanized steel sheet was visually observed, and the presence or absence of a region where plating did not exist and the steel sheet was exposed (the presence or absence of a bare spot defect) was investigated by the order of approximately several micrometers to several millimeters. As a result of the investigation, it has been found that this galvanized steel sheet does not have a bare spot defect and has good plating ability.

TABLE 2

| Steel No. | Chemical composition (mass %) |      |      |       |        |        |       | Ac3 (° C.)                                | Si/Mn (Mass ratio) | Remarks |                   |
|-----------|-------------------------------|------|------|-------|--------|--------|-------|-------------------------------------------|--------------------|---------|-------------------|
|           | C                             | Si   | Mn   | P     | S      | N      | Al    |                                           |                    |         |                   |
| A         | 0.123                         | 0.30 | 2.65 | 0.008 | 0.0008 | 0.0035 | 0.040 | Ti: 0.022, Nb: 0.024                      | 798                | 0.11    | Conforming steel  |
| B         | 0.090                         | 0.50 | 3.25 | 0.006 | 0.0007 | 0.0030 | 0.035 | Ti: 0.015, Nb: 0.015                      | 794                | 0.15    | Conforming steel  |
| C         | 0.145                         | 0.40 | 2.50 | 0.007 | 0.0008 | 0.0030 | 0.033 | —                                         | 789                | 0.16    | Conforming steel  |
| D         | 0.188                         | 0.40 | 2.50 | 0.007 | 0.0016 | 0.0030 | 0.033 | —                                         | 779                | 0.16    | Conforming steel  |
| E         | 0.123                         | 0.65 | 3.44 | 0.015 | 0.0008 | 0.0030 | 0.033 | —                                         | 778                | 0.19    | Conforming steel  |
| F         | 0.123                         | 0.30 | 1.64 | 0.007 | 0.0008 | 0.0050 | 0.033 | —                                         | 817                | 0.18    | Conforming steel  |
| G         | 0.123                         | 0.40 | 2.50 | 0.007 | 0.0008 | 0.0030 | 0.080 | Ti: 0.021, Nb: 0.025, V: 0.005, Zr: 0.010 | 823                | 0.16    | Conforming steel  |
| H         | 0.123                         | 0.40 | 2.50 | 0.007 | 0.0008 | 0.0030 | 0.033 | Mo: 0.11, Cr: 0.22                        | 795                | 0.16    | Conforming steel  |
| I         | 0.145                         | 0.40 | 2.50 | 0.007 | 0.0008 | 0.0030 | 0.033 | Sb: 0.010, Sn: 0.02                       | 789                | 0.16    | Conforming steel  |
| J         | 0.115                         | 0.44 | 2.50 | 0.007 | 0.0008 | 0.0030 | 0.033 | Ca: 0.0003                                | 800                | 0.18    | Conforming steel  |
| K         | 0.123                         | 0.10 | 2.50 | 0.007 | 0.0008 | 0.0030 | 0.033 | —                                         | 782                | 0.04    | Comparative steel |
| L         | 0.123                         | 1.00 | 3.70 | 0.007 | 0.0009 | 0.0030 | 0.033 | —                                         | 786                | 0.27    | Comparative steel |
| M         | 0.060                         | 0.40 | 2.50 | 0.007 | 0.0008 | 0.0030 | 0.033 | —                                         | 817                | 0.16    | Comparative steel |
| N         | 0.230                         | 0.40 | 2.50 | 0.007 | 0.0008 | 0.0030 | 0.033 | —                                         | 769                | 0.16    | Comparative steel |
| O         | 0.123                         | 2.10 | 2.50 | 0.007 | 0.0008 | 0.0030 | 0.033 | —                                         | 871                | 0.84    | Comparative steel |
| P         | 0.123                         | 0.20 | 1.20 | 0.007 | 0.0008 | 0.0030 | 0.033 | —                                         | 825                | 0.17    | Comparative steel |
| Q         | 0.123                         | 0.40 | 2.50 | 0.007 | 0.0030 | 0.0030 | 0.033 | —                                         | 797                | 0.16    | Comparative steel |
| R         | 0.123                         | 0.40 | 2.50 | 0.007 | 0.0008 | 0.0090 | 0.033 | —                                         | 795                | 0.16    | Comparative steel |
| S         | 0.123                         | 0.40 | 2.50 | 0.007 | 0.0008 | 0.0030 | 0.200 | —                                         | 862                | 0.16    | Comparative steel |

TABLE 3

| No. | Steel No. | Casting Flow velocity of molten steel *1 (cm/s) | Cold rolling | Annealing | In-furnace |                   |                    | Average cooling rate Annealing |                                                                      |    |
|-----|-----------|-------------------------------------------------|--------------|-----------|------------|-------------------|--------------------|--------------------------------|----------------------------------------------------------------------|----|
|     |           |                                                 |              |           | Steel No.  | Rolling ratio (%) | temperature (° C.) | Hydrogen concentration (vol %) | Dew-point temperature (temperature region of 750° C. or more) (° C.) |    |
|     |           |                                                 |              |           |            |                   |                    |                                |                                                                      |    |
| 1   | A         | 22                                              | 45           | 815       | 5          |                   |                    | -45                            | 4                                                                    | 50 |
| 2   | B         | 18                                              | 50           | 800       | 9          |                   |                    | -50                            | 5                                                                    | 50 |
| 3   | B         | 21                                              | 50           | 800       | 9          |                   |                    | -50                            | 5                                                                    | 50 |
| 4   | A         | 22                                              | 50           | 800       | 8          |                   |                    | -50                            | 5                                                                    | 50 |
| 5   | B         | 10                                              | 50           | 800       | 9          |                   |                    | -50                            | 5                                                                    | 50 |
| 6   | B         | 18                                              | 50           | 780       | 9          |                   |                    | -45                            | 5                                                                    | 50 |
| 7   | B         | 18                                              | 50           | 700       | 9          |                   |                    | -45                            | 5                                                                    | 50 |
| 8   | B         | 18                                              | 50           | 840       | 9          |                   |                    | -45                            | 5                                                                    | 50 |
| 9   | B         | 18                                              | 50           | 780       | 15         |                   |                    | -45                            | 5                                                                    | 50 |
| 10  | B         | 18                                              | 50           | 780       | 0.5        |                   |                    | -45                            | 5                                                                    | 50 |
| 11  | B         | 18                                              | 50           | 780       | 10         |                   |                    | -45                            | 5                                                                    | 10 |
| 12  | B         | 18                                              | 50           | 750       | 8          |                   |                    | -45                            | 1                                                                    | 50 |
| 13  | B         | 16                                              | 50           | 780       | 8          |                   |                    | -45                            | 5                                                                    | 50 |
| 14  | B         | 18                                              | 50           | 780       | 1          |                   |                    | -45                            | 5                                                                    | 50 |
| 15  | B         | 18                                              | 50           | 780       | 8          |                   |                    | -45                            | 3                                                                    | 50 |
| 16  | B         | 18                                              | 50           | 780       | 8          |                   |                    | -45                            | 5                                                                    | 50 |
| 17  | B         | 18                                              | 50           | 780       | 8          |                   |                    | -45                            | 5                                                                    | 50 |
| 18  | B         | 18                                              | 50           | 780       | 8          |                   |                    | -45                            | 5                                                                    | 50 |
| 19  | B         | 18                                              | 50           | 780       | 8          |                   |                    | -45                            | 5                                                                    | 50 |
| 20  | C         | 18                                              | 50           | 780       | 8          |                   |                    | -45                            | 4                                                                    | 50 |
| 21  | D         | 18                                              | 50           | 780       | 8          |                   |                    | -45                            | 5                                                                    | 50 |

TABLE 3-continued

| No. | Plating<br>450 to 250° C.<br>(° C./s) | Width<br>*2 | Post-treatment         |                                      |                                    |                       |               |                     | Remarks |
|-----|---------------------------------------|-------------|------------------------|--------------------------------------|------------------------------------|-----------------------|---------------|---------------------|---------|
|     |                                       |             | Presence<br>or absence | Hydrogen<br>concentration<br>(vol %) | Dew-point<br>temperature<br>(° C.) | Temperature<br>(° C.) | Time<br>(min) | Remarks             |         |
| 1   | 5                                     | Absence     | 0                      | 0                                    | 100                                | 2880                  |               | Invented example    |         |
| 2   | 6                                     | Absence     | —                      | —                                    | —                                  | —                     |               | Invented example    |         |
| 3   | 6                                     | Absence     | 0                      | 0                                    | 50                                 | 5                     |               | Invented example    |         |
| 4   | 10                                    | Absence     | —                      | —                                    | —                                  | —                     |               | Invented example    |         |
| 5   | 6                                     | Absence     | —                      | —                                    | —                                  | —                     |               | Comparative example |         |
| 6   | 6                                     | Absence     | —                      | —                                    | —                                  | —                     |               | Invented example    |         |
| 7   | 6                                     | Absence     | —                      | —                                    | —                                  | —                     |               | Comparative example |         |
| 8   | 6                                     | Absence     | —                      | —                                    | —                                  | —                     |               | Comparative example |         |
| 9   | 6                                     | Absence     | —                      | —                                    | —                                  | —                     |               | Comparative example |         |
| 10  | 6                                     | Absence     | —                      | —                                    | —                                  | —                     |               | Invented example    |         |
| 11  | 6                                     | Absence     | —                      | —                                    | —                                  | —                     |               | Comparative example |         |
| 12  | 6                                     | Absence     | —                      | —                                    | —                                  | —                     |               | Comparative example |         |
| 13  | 6                                     | Absence     | —                      | —                                    | —                                  | —                     |               | Invented example    |         |
| 14  | 6                                     | Absence     | —                      | —                                    | —                                  | —                     |               | Invented example    |         |
| 15  | 6                                     | Absence     | —                      | —                                    | —                                  | —                     |               | Invented example    |         |
| 16  | 3                                     | Absence     | —                      | —                                    | —                                  | —                     |               | Invented example    |         |
| 17  | 6                                     | Presence    | —                      | —                                    | —                                  | —                     |               | Invented example    |         |
| 18  | 6                                     | Absence     | 5                      | 0                                    | 100                                | 120                   |               | Invented example    |         |
| 19  | 6                                     | Absence     | 15                     | 0                                    | 100                                | 120                   |               | Invented example    |         |
| 20  | 6                                     | Absence     | —                      | —                                    | —                                  | —                     |               | Invented example    |         |
| 21  | 6                                     | Absence     | —                      | —                                    | —                                  | —                     |               | Invented example    |         |
| 22  | 6                                     | Absence     | —                      | —                                    | —                                  | —                     |               | Invented example    |         |
| 23  | 8                                     | Absence     | —                      | —                                    | —                                  | —                     |               | Invented example    |         |
| 24  | 8                                     | Absence     | —                      | —                                    | —                                  | —                     |               | Comparative example |         |
| 25  | 2                                     | Absence     | —                      | —                                    | —                                  | —                     |               | Comparative example |         |
| 26  | 6                                     | Absence     | —                      | —                                    | —                                  | —                     |               | Invented example    |         |
| 27  | 6                                     | Absence     | —                      | —                                    | —                                  | —                     |               | Invented example    |         |
| 28  | 6                                     | Absence     | —                      | —                                    | —                                  | —                     |               | Invented example    |         |
| 29  | 6                                     | Absence     | —                      | —                                    | —                                  | —                     |               | Invented example    |         |
| 30  | 6                                     | Absence     | —                      | —                                    | —                                  | —                     |               | Comparative example |         |
| 31  | 6                                     | Absence     | —                      | —                                    | —                                  | —                     |               | Comparative example |         |
| 32  | 10                                    | Absence     | —                      | —                                    | —                                  | —                     |               | Comparative example |         |
| 33  | 10                                    | Absence     | —                      | —                                    | —                                  | —                     |               | Comparative example |         |
| 34  | 6                                     | Absence     | —                      | —                                    | —                                  | —                     |               | Comparative example |         |
| 35  | 6                                     | Absence     | —                      | —                                    | —                                  | —                     |               | Comparative example |         |
| 36  | 6                                     | Absence     | —                      | —                                    | —                                  | —                     |               | Comparative example |         |
| 37  | 6                                     | Absence     | —                      | —                                    | —                                  | —                     |               | Comparative example |         |
| 38  | 6                                     | Absence     | —                      | —                                    | —                                  | —                     |               | Comparative example |         |

\*1 A flow velocity of molten steel at a solidification interface in vicinity of a meniscus of a casting mold

\*2 An average cooling rate from 450° C. to 250° C. after the plating treatment

\*3: The retention time for temperature region of 500° C. to 400° C.

TABLE 4

| No. | Steel No. | Product sheet           |                               |                                       |                            | Steel structure                          |                 |                         |
|-----|-----------|-------------------------|-------------------------------|---------------------------------------|----------------------------|------------------------------------------|-----------------|-------------------------|
|     |           | Inclusions *1           |                               | Coating weight *2 (g/m <sup>2</sup> ) | Plating ability evaluation | Amount of diffusible hydrogen (Mass ppm) | F               |                         |
|     |           | Average grain size (μm) | Average nearest distance (μm) |                                       |                            |                                          | Area ratios (%) | Average grain size (μm) |
| 1   | A         | 40                      | 55                            | 40                                    | A                          | 0.12                                     | 30              | 8                       |
| 2   | B         | 30                      | 50                            | 55                                    | A                          | 0.11                                     | 35              | 8                       |
| 3   | B         | 15                      | 100                           | 50                                    | A                          | 0.06                                     | 35              | 8                       |
| 4   | A         | 15                      | 80                            | 50                                    | A                          | 0.19                                     | 5               | 3                       |
| 5   | B         | 50                      | 15                            | 50                                    | A                          | 0.13                                     | 35              | 8                       |
| 6   | B         | 25                      | 55                            | 55                                    | A                          | 0.22                                     | 10              | 5                       |
| 7   | B         | 30                      | 50                            | 60                                    | A                          | 0.09                                     | 100             | 14                      |
| 8   | B         | 25                      | 55                            | 55                                    | A                          | 0.37                                     | 0               | —                       |
| 9   | B         | 30                      | 50                            | 55                                    | A                          | 0.44                                     | 50              | 10                      |
| 10  | B         | 25                      | 55                            | 45                                    | C                          | 0.05                                     | 10              | 5                       |
| 11  | B         | 25                      | 55                            | 45                                    | D                          | 0.26                                     | 10              | 5                       |
| 12  | B         | 25                      | 55                            | 55                                    | A                          | 0.11                                     | 100             | 30                      |
| 13  | B         | 43                      | 30                            | 55                                    | A                          | 0.20                                     | 10              | 5                       |
| 14  | B         | 25                      | 55                            | 45                                    | B                          | 0.08                                     | 10              | 5                       |
| 15  | B         | 25                      | 55                            | 50                                    | A                          | 0.18                                     | 15              | 8                       |
| 16  | B         | 25                      | 55                            | 50                                    | A                          | 0.18                                     | 10              | 5                       |
| 17  | B         | 25                      | 55                            | 45                                    | A                          | 0.10                                     | 10              | 5                       |
| 18  | B         | 25                      | 55                            | 50                                    | A                          | 0.12                                     | 10              | 5                       |
| 19  | B         | 25                      | 55                            | 45                                    | A                          | 0.20                                     | 10              | 5                       |
| 20  | C         | 28                      | 52                            | 55                                    | A                          | 0.20                                     | 5               | 3                       |
| 21  | D         | 37                      | 29                            | 50                                    | A                          | 0.21                                     | 3               | 2                       |
| 22  | E         | 33                      | 46                            | 45                                    | B                          | 0.21                                     | 3               | 2                       |
| 23  | F         | 20                      | 63                            | 55                                    | A                          | 0.18                                     | 30              | 8                       |
| 24  | F         | 20                      | 63                            | 55                                    | A                          | 0.12                                     | 40              | 25                      |
| 25  | F         | 20                      | 63                            | 55                                    | A                          | 0.14                                     | 30              | 8                       |
| 26  | G         | 35                      | 30                            | 50                                    | A                          | 0.18                                     | 35              | 8                       |
| 27  | H         | 25                      | 47                            | 55                                    | A                          | 0.17                                     | 15              | 5                       |
| 28  | I         | 30                      | 50                            | 50                                    | A                          | 0.13                                     | 5               | 3                       |
| 29  | J         | 25                      | 60                            | 55                                    | A                          | 0.16                                     | 35              | 15                      |
| 30  | K         | 30                      | 50                            | 50                                    | D                          | 0.19                                     | 15              | 5                       |
| 31  | L         | 33                      | 50                            | 45                                    | D                          | 0.13                                     | 2               | 2                       |
| 32  | M         | 15                      | 73                            | 55                                    | A                          | 0.17                                     | 25              | 10                      |
| 33  | N         | 35                      | 50                            | 55                                    | A                          | 0.21                                     | 0               | —                       |
| 34  | O         | 40                      | 35                            | 45                                    | D                          | 0.19                                     | 40              | 15                      |
| 35  | P         | 15                      | 61                            | 55                                    | A                          | 0.18                                     | 35              | 8                       |
| 36  | Q         | 30                      | 23                            | 55                                    | A                          | 0.18                                     | 35              | 8                       |
| 37  | R         | 30                      | 54                            | 50                                    | D                          | 0.19                                     | 35              | 8                       |
| 38  | S         | 84                      | 20                            | 55                                    | A                          | 0.21                                     | 35              | 8                       |

  

| No. | Steel structure |                 |                 |          |                 |                     | Remarks |  |
|-----|-----------------|-----------------|-----------------|----------|-----------------|---------------------|---------|--|
|     | B               |                 | Retained γ      |          | Others          |                     |         |  |
|     | Area ratios (%) | Area ratios (%) | Area ratios (%) | TS (MPa) | Bendability R/t | Remarks             |         |  |
| 1   | 10              | 4               | 1               | 1220     | 2.1             | Invented example    |         |  |
| 2   | 10              | 0               | 0               | 1210     | 2.5             | Invented example    |         |  |
| 3   | 10              | 0               | 0               | 1205     | 1.4             | Invented example    |         |  |
| 4   | 20              | 0               | 0               | 1260     | 2.3             | Invented example    |         |  |
| 5   | 10              | 0               | 0               | 1215     | 5.3             | Comparative example |         |  |
| 6   | 20              | 2               | 0               | 1230     | 2.5             | Invented example    |         |  |
| 7   | 0               | 0               | 0               | 850      | 1.1             | Comparative example |         |  |
| 8   | 25              | 2               | 0               | 1220     | 4.0             | Comparative example |         |  |
| 9   | 5               | 0               | 0               | 1200     | 4.6             | Comparative example |         |  |
| 10  | 20              | 2               | 0               | 1230     | 1.8             | Invented example    |         |  |
| 11  | 10              | 0               | 0               | 1250     | 2.7             | Comparative example |         |  |
| 12  | 0               | 0               | 0               | 800      | 0.7             | Comparative example |         |  |
| 13  | 20              | 2               | 0               | 1230     | 3.4             | Invented example    |         |  |
| 14  | 20              | 2               | 0               | 1230     | 2.1             | Invented example    |         |  |
| 15  | 15              | 1               | 5               | 1205     | 2.2             | Invented example    |         |  |
| 16  | 35              | 1               | 5               | 1130     | 2.5             | Invented example    |         |  |
| 17  | 20              | 0               | 0               | 1230     | 2.0             | Invented example    |         |  |
| 18  | 20              | 0               | 0               | 1220     | 2.1             | Invented example    |         |  |
| 19  | 20              | 0               | 0               | 1220     | 2.5             | Invented example    |         |  |
| 20  | 25              | 2               | 0               | 1180     | 2.5             | Invented example    |         |  |
| 21  | 25              | 1               | 2               | 1315     | 2.8             | Invented example    |         |  |
| 22  | 30              | 0               | 2               | 1350     | 2.6             | Invented example    |         |  |
| 23  | 10              | 0               | 0               | 1170     | 2.2             | Invented example    |         |  |
| 24  | 15              | 0               | 10              | 985      | 1.1             | Comparative example |         |  |
| 25  | 25              | 1               | 0               | 1073     | 1.4             | Comparative example |         |  |

TABLE 4-continued

|    |    |   |   |      |     |                     |
|----|----|---|---|------|-----|---------------------|
| 26 | 5  | 0 | 0 | 1280 | 3.2 | Invented example    |
| 27 | 5  | 0 | 0 | 1240 | 2.5 | Invented example    |
| 28 | 25 | 2 | 0 | 1185 | 2.5 | Invented example    |
| 29 | 5  | 0 | 0 | 1150 | 2.1 | Invented example    |
| 30 | 10 | 0 | 0 | 1180 | 2.5 | Comparative example |
| 31 | 5  | 0 | 3 | 1475 | 2.5 | Comparative example |
| 32 | 5  | 0 | 0 | 1000 | 2.2 | Comparative example |
| 33 | 10 | 0 | 0 | 1490 | 4.5 | Comparative example |
| 34 | 10 | 0 | 0 | 1170 | 3.0 | Comparative example |
| 35 | 10 | 0 | 0 | 1030 | 2.5 | Comparative example |
| 36 | 10 | 0 | 0 | 1180 | 4.1 | Comparative example |
| 37 | 10 | 0 | 0 | 1190 | 2.5 | Comparative example |
| 38 | 10 | 0 | 0 | 1180 | 3.7 | Comparative example |

\*1 Inclusions containing at least one of Al, Si, Mg, and Ca and existing in an area extending from a surface to a position of  $\frac{1}{3}$  of a sheet thickness

\*2 A coating weight per one surface of a steel sheet

F: Ferrite, M: Martensite, B: Bainite, Retained  $\gamma$ : Retained austenite

The galvanized steel sheets of Present Invention Examples obtained by means of components and manufacturing conditions in the ranges according to aspects of the present invention had  $TS \geq 1100$  MPa or more, which indicates high strength, had  $R/t \leq 3.5$ , which indicates excellent bendability, and was excellent in plating ability. On the other hand, in the galvanized steel sheets of the Comparative Examples, at least one of these properties was poorer than in the Present Invention Examples.

### Example 3

A galvanized steel sheet of manufacturing conditions No. 1 (Present Invention Example) of Table 3 of Example 2 was press-formed to manufacture a member of a Present Invention Example. Further, a galvanized steel sheet of manufacturing conditions No. 1 (Present Invention Example) of Table 3 of Example 2 and a galvanized steel sheet of manufacturing conditions No. 2 (Present Invention Example) of Table 3 of Example 2 were joined together by spot welding to manufacture a member of a Present Invention Example. It has been verified that these members of Present Invention Examples are excellent in bendability and plating ability and can therefore be suitably used for automotive parts or the like.

### INDUSTRIAL APPLICABILITY

The high-strength galvanized steel sheet according to embodiments of the present invention has not only a high tensile strength but also good bendability and good plating ability. Therefore, the high-strength galvanized steel sheet according to embodiments of the present invention contributes to environment conservation, for example, from the viewpoint of  $CO_2$  emission by contributing to an improvement in safety performance and to a decrease in the weight of an automobile body through an improvement in strength and a decrease in thickness, in the case where the steel sheet is used for the frame members, in particular, for the parts around a cabin, which has an influence on crash safety, of an automobile body. In addition, since the steel sheet has both good surface quality and coating quality, it is possible to actively use for parts such as chassis which are prone to corrosion due to rain or snow, and it is also possible to expect an improvement in the rust prevention capability and corrosion resistance of an automobile body. A material having such properties can effectively be used not only for automotive parts but also in the industrial fields of civil engineering, construction, and home electrical appliances.

The invention claimed is:

1. A high-strength galvanized steel sheet comprising: a steel sheet having a chemical composition containing a steel composition containing, in mass %, C: 0.08% or more and 0.20% or less, Si: less than 2.0%, Mn: 1.5% or more and 3.5% or less, P: 0.02% or less, S: 0.002% or less, Al: 0.10% or less, and N: 0.006% or less,

a mass ratio of a content of Si to a content of Mn in the steel (Si/Mn) being 0.1 or more and less than 0.2, and the balance: Fe and incidental impurities, and

a steel structure in which an average grain size of inclusions containing at least one of Al, Si, Mg, and Ca and existing in an area extending from a surface to a position of  $\frac{1}{3}$  of a sheet thickness is 50  $\mu m$  or less, and an average nearest distance between the inclusions is 20  $\mu m$  or more; and

a galvanized layer provided on a surface of the steel sheet and having a coating weight per one surface of 20  $g/m^2$  or more and 120  $g/m^2$  or less,

wherein an amount of diffusible hydrogen contained in the steel sheet is less than 0.25 mass ppm, and a tensile strength is 1100 MPa or more,

and wherein the steel structure contains 40% or more and 90% or less of martensite, 35% or less (including 0%) of ferrite, 50% or less (including 0%) of bainite, and less than 3% (including 0%) of retained austenite in terms of area ratio, and

an average grain size of ferrite is 25  $\mu m$  or less.

2. The high-strength galvanized steel sheet according to claim 1, wherein the chemical composition further contains, in mass %, at least one of (1) to (5) below,

- (1) one or more of Ti, Nb, V, and Zr: 0.005% or more and 0.1% or less in total,
- (2) one or more of Mo, Cr, Cu, and Ni: 0.01% or more and 0.5% or less in total,
- (3) B: 0.0003% or more and 0.005% or less,
- (4) at least one of Sb: 0.001% or more and 0.1% or less and Sn: 0.001% or more and 0.1% or less, and
- (5) Ca: 0.0005% or less.

3. A method for manufacturing the high-strength galvanized steel sheet according to claim 1, comprising: a casting step of casting steel having the chemical composition under a condition where a flow velocity of molten steel at a solidification interface in vicinity of a meniscus of a casting mold is 16 cm/s or more, and producing a steel raw material;

## 27

a hot rolling step of hot rolling the steel raw material after the casting step, thereby producing a steel sheet; a pickling step of pickling the steel sheet after the hot rolling step; a cold rolling step of cold rolling the steel sheet after the pickling step at a rolling reduction ratio of 20% or more and 80% or less; an annealing step of heating the steel sheet after the cold rolling step in a continuous annealing line at an annealing temperature of  $(Ac3-30)^\circ C$ . or more and  $(Ac3+20)^\circ C$ . or less, with a hydrogen concentration of an atmosphere in a furnace of  $500^\circ C$ . or more set to more than 0 vol % and less than 10 vol % and a dew-point temperature of an atmosphere in the furnace of  $750^\circ C$ . or more set to  $-45^\circ C$ . or less, then performing cooling at an average cooling rate of  $3^\circ C/s$  or more from the annealing temperature to at least  $600^\circ C$ ., and then performing retaining in a temperature region of  $500^\circ C$ . to  $400^\circ C$ . for 45 seconds or more; and a plating step of subjecting the steel sheet after the annealing step to plating treatment, and after the plating treatment, performing cooling at an average cooling rate of  $3^\circ C/s$  or more through a temperature region of  $450^\circ C$ . to  $250^\circ C$ .

4. A method for manufacturing the high-strength galvanized steel sheet according to claim 2, comprising:

a casting step of casting steel having the chemical composition under a condition where a flow velocity of molten steel at a solidification interface in vicinity of a meniscus of a casting mold is 16 cm/s or more, and producing a steel raw material; a hot rolling step of hot rolling the steel raw material after the casting step, thereby producing a steel sheet; a pickling step of pickling the steel sheet after the hot rolling step; a cold rolling step of cold rolling the steel sheet after the pickling step at a rolling reduction ratio of 20% or more and 80% or less; an annealing step of heating the steel sheet after the cold rolling step in a continuous annealing line at an annealing temperature of  $(Ac3-30)^\circ C$ . or more and  $(Ac3+20)^\circ C$ . or less, with a hydrogen concentration of an atmosphere in a furnace of  $500^\circ C$ . or more set to more than 0 vol % and less than 10 vol % and a dew-point temperature of an atmosphere in the furnace of  $750^\circ C$ . or more set to  $-45^\circ C$ . or less, then performing cooling at an average cooling rate of  $3^\circ C/s$  or more from the annealing temperature to at least  $600^\circ C$ ., and then performing retaining in a temperature region of  $500^\circ C$ . to  $400^\circ C$ . for 45 seconds or more; and a plating step of subjecting the steel sheet after the annealing step to plating treatment, and after the plating

## 28

treatment, performing cooling at an average cooling rate of  $3^\circ C/s$  or more through a temperature region of  $450^\circ C$ . to  $250^\circ C$ .

5. The method according to claim 3, wherein the step further comprises at least one of (1) and (2) below,

- (1) after the plating step, a width trimming step of performing width trimming, and
- (2) after the annealing step or after the plating step, a post-treatment step of performing heating in a temperature region of 50 to  $400^\circ C$ . for 30 seconds or more in an atmosphere with a hydrogen concentration of 5 vol % or less and a dew-point temperature of  $50^\circ C$ . or less.

6. The method according to claim 4, wherein the step further comprises at least one of (1) and (2) below,

- (1) after the plating step, a width trimming step of performing width trimming, and
- (2) after the annealing step or after the plating step, a post-treatment step of performing heating in a temperature region of 50 to  $400^\circ C$ . for 30 seconds or more in an atmosphere with a hydrogen concentration of 5 vol % or less and a dew-point temperature of  $50^\circ C$ . or less.

7. The method according to claim 3, wherein alloying treatment is performed immediately after the plating treatment in the plating step.

8. The method according to claim 4, wherein alloying treatment is performed immediately after the plating treatment in the plating step.

9. The method according to claim 5, wherein alloying treatment is performed immediately after the plating treatment in the plating step.

10. The method according to claim 6, wherein alloying treatment is performed immediately after the plating treatment in the plating step.

11. A method for manufacturing a high strength member, comprising a step of performing at least either one of forming and welding on the high-strength galvanized steel sheet according to claim 1.

12. A method for manufacturing a high strength member, comprising a step of performing at least either one of forming and welding on the high-strength galvanized steel sheet according to claim 2.

13. The high-strength galvanized steel sheet according to claim 1, wherein plating peeling resistance represented by a counted number of Zn pieces is less than 8000, where the counted number of Zn pieces is measured such that a cellophane tape is pressed against a processed portion of the hot-dip galvanized steel sheet where bending of  $90^\circ$  is performed, peeled substances are transferred to the cellophane tape, and the amount of peeled substances on the cellophane tape is found as the counted number of Zn pieces by an X-ray fluorescence method.

\* \* \* \* \*